



US006156490A

# United States Patent [19]

Slusarek et al.

[11] Patent Number: 6,156,490

[45] Date of Patent: Dec. 5, 2000

[54] **PHOTOGRAPHIC ELEMENT CONTAINING A STABLE ARYLOXYPYRAZOLONE COUPLER AND PROCESS EMPLOYING SAME**

[75] Inventors: **Wojciech K. Slusarek; Jerrold N. Poslusny**, both of Rochester; **Xiqiang K. Yang**, Webster, all of N.Y.

[73] Assignee: **Eastman Kodak Company**, Rochester, N.Y.

[\*] Notice: This patent is subject to a terminal disclaimer.

[21] Appl. No.: 09/224,252

[22] Filed: **Dec. 30, 1998**

[51] **Int. Cl.<sup>7</sup>** ..... G03C 1/08; G03C 7/26; G03C 7/32

[52] **U.S. Cl.** ..... 430/555; 430/544; 430/955; 430/956; 430/957; 430/958; 430/959; 430/960

[58] **Field of Search** ..... 430/555, 544, 430/955, 956, 957, 958, 959, 960

## [56] References Cited

### U.S. PATENT DOCUMENTS

|           |         |                 |       |         |
|-----------|---------|-----------------|-------|---------|
| 3,419,391 | 12/1968 | Young           | ..... | 430/543 |
| 4,686,175 | 8/1987  | Ogawa et al.    | ..... | 430/555 |
| 4,985,336 | 1/1991  | Ichijima et al. | ..... | 430/505 |
| 5,567,167 | 10/1996 | Poslusny et al. | ..... | 430/555 |
| 5,670,308 | 9/1997  | Poslusny et al. | ..... | 430/555 |

Primary Examiner—Geraldine Letscher  
Attorney, Agent, or Firm—Arthur E. Kluegel

## [57] ABSTRACT

Disclosed is a photographic element comprising a light-sensitive silver halide emulsion layer having associated

therewith a coupler based on a 1-aryl-3-arylpyrazol-5-one or a 1-aryl-3-alkylpyrazol-5-one ring and represented by formula I:

I



wherein:

X represents an aryl, alkyl, alkylamino, or arylamino group;

Y can be carbon or sulfur; in is 1 when Y is carbon and 2 when Y is sulfur;

R represents a halogen or an alkyl group; and o is 0 to 4, provided that two or more R substituents may join to form one or more additional rings;

Z is either (a) an aryl group represented as Ar<sup>3</sup>Q(n) where Q represents n independently selected substituents bonded to the Ar<sup>3</sup> ring; and n is 0 to 5, provided that two or more Q substituents may join to form one or more additional rings or (b) an alkyl group;

OAr<sup>4</sup> is an aryloxy group; and

P represents p independently selected substituents bonded to the OAr<sup>4</sup> aryloxy ring, provided that P may not be a nitro group ortho to the oxygen atom linking the aryloxy group to the 4-position of the pyrazolone ring; and p is 0 to 5, provided that two or more P substituents may join to form one or more additional rings;

provided that X and an R group may join to form an additional ring.

**20 Claims, No Drawings**

**PHOTOGRAPHIC ELEMENT CONTAINING  
A STABLE ARYLOXYPYRAZOLONE  
COUPLER AND PROCESS EMPLOYING  
SAME**

**FIELD OF THE INVENTION**

This invention relates to a photographic element having a light-sensitive silver halide emulsion layer having associated therewith a stable 1-aryl-3-arylpypyrazol-5-one or 1-aryl-3-alkylpyrazol-5-one based magenta coupler having an aryloxy group linked by its oxygen atom to the 4- position of the pyrazolone ring.

**BACKGROUND OF THE INVENTION**

In a silver halide photographic element, a color image is formed when the material is exposed to light and then developed using a primary amine color developer. The development results in imagewise reduction of silver halide and the corresponding production of oxidized developer. The oxidized developer then reacts in an imagewise fashion with one or more incorporated dye-forming couplers to form a dye image.

Magenta dye-forming couplers are employed in subtractive color forming processes. One of the principal coupler types useful for this purpose are those based on a pyrazolone ring. Pyrazolone-based couplers having a coupling-off group linked to the pyrazolone ring by oxygen have long been considered as potentially attractive two equivalent magenta couplers. An oxygen-linked coupling-off group could impart increased activity to the pyrazolone coupler; however the general instability of these couplers toward ambient oxygen makes them difficult to synthesize and impractical for use in a film environment since they decompose during keeping. In particular, pyrazolone couplers having an anilino or acylamino substituent at the 3-position have exhibited unacceptable stability when an aryloxy is employed as a coupling-off group. As a result, pyrazolone couplers have employed either so-called "four equivalent" couplers containing hydrogen at the coupling-off position or have employed so-called "two-equivalent" couplers containing a coupling-off group having a sulfur or nitrogen atom linked to the pyrazolone ring.

U.S. Pat. No. 3,419,391 discloses certain types of pyrazolone-based compounds as two-equivalent couplers having high dye-forming reactivity and reduced tendency to form color fog. According to the patent, the pyrazolone ring is not limited to the presence of any particular substituents at the 3-position or elsewhere. Specifically identified substituents at the 3-position include anilino, acylamino, alkyl, amino, alkoxy, amido, carbamoyl, ureido, thio, guanidino, etc. The couplers of the patent may contain an aryl group at the 1-position and, among other things, an alkyl or carboxy ester group at the 3-position. The aryloxy couplers of the patent are said not to produce color fog (printout) and to provide improved reactivity. Thus, they are said to provide low printout or yellowing in Dmin areas when they are exposed to light or high temperatures, respectively, subsequent to development. No mention is made of the poor keeping of pyrazolone couplers having aryloxy coupling-off groups although their instability is well known in the art.

U.S. Pat. No. 5,576,167 describes a family of two-equivalent pyrazolone couplers with good stability towards oxygen. The features that make these compounds stable are: (a) an electron-withdrawing CXYZ substituent in the 3-position of the pyrazolone ring, and (b) an aryloxy group, further substituted by electron-withdrawing group(s) in the

4-position of the ring. Although stable, the couplers of this patent require a multistep procedure for their preparation and some of these steps are difficult to perform. None of these references discloses magenta couplers of this invention.

In a co-pending application we describe 1-aryl-3-arylpypyrazol-5-one magenta dye forming couplers that are stable during synthesis, film manufacture, and during film keeping and are not difficult to prepare. However, in general, 10 these couplers are not crystalline and therefore difficult to manufacture.

It would be desirable to have magenta dye forming couplers of the 1-aryl-3-arylpypyrazol-5-one and/or the 1-aryl-3-alkylpyrazol-5-one type that are stable during 15 synthesis, film manufacture, and during film keeping that would provide acceptable hue and reactivity but which would be crystalline.

**SUMMARY OF THE INVENTION**

The invention provides a photographic element comprising a light-sensitive silver halide emulsion layer having associated therewith a coupler based on a 1-aryl-3-arylpypyrazol-5-one or a 1-aryl-3-alkylpyrazol-5-one ring and represented by formula I:



wherein:

X represents an aryl, alkyl, alkylamino, or arylamino group;

Y can be carbon or sulfur; m is 1 when Y is carbon and 2 when Y is sulfur;

R represents a halogen or an alkyl group; and o is 0 to 4, provided that two or more R substituents may join to form one or more additional rings;

Z is either (a) an aryl group represented as Ar^3Q(n) where Q represents n independently selected substituents bonded to the Ar^3 ring; and n is 0 to 5, provided that two or more Q substituents may join to form one or more additional rings or (b) an alkyl group;

OAr^4 is an aryloxy group; and

P represents p independently selected substituents bonded to the OAr^4 aryloxy ring, provided that P may not be a nitro group ortho to the oxygen atom linking the aryloxy group to the 4-position of the pyrazolone ring; and p is 0 to 5, provided that two or more P substituents may join to form one or more additional rings;

provided that X and an R group may join to form an additional ring.

The invention also encompasses a process for forming an image in the described element after exposure to light comprising contacting the element with a color developing chemical.

A photographic element in accordance with the invention exhibits an improved keeping stability of the magenta dye forming coupler and acceptable hue and reactivity even in the absence of a stabilizing compound.

## DETAILED DESCRIPTION OF THE INVENTION

The aryl group identified at the 1-position, the aryl or alkyl group identified at the 3-position, and the aryloxy group identified at the 4-position of the pyrazolone ring are independently selected.

It is essential that the 4-aryloxy group not include a nitro group ortho to the oxygen atom linking 4-aryloxy to the pyrazolone ring. The exclusion of ortho nitro on 4-aryloxy is necessitated by its very strong destabilizing effect on the corresponding pyrazolone couplers which leads to their very rapid decomposition.

Also within the scope of the invention are couplers which release a photographically useful group (PUG). PUG can be any photographically useful group known in the art. For example, PUG can be a dye or dye precursor, such as a sensitizing dye, filter dye, image dye, leuco dye, blocked dye, shifted dye, or ultraviolet light absorber. Alternatively PUG can be a photographic reagent, which upon release can further react with components in the element. Such reagents include development accelerators or inhibitors, bleach accelerators or inhibitors, couplers (e.g. competing couplers, color-forming couplers, or DIR couplers), developing agents (e.g. competing developing agents or auxiliary developing agents), silver complexing agents, fixing agents, toners, hardeners, tanning agents, fogging agents, antifoggants, antistain agents, stabilizers, nucleophiles and dinucleophiles, and chemical or spectral sensitizers and desensitizers.

Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzisodiazoles. In a preferred embodiment, the inhibitor moiety or group is selected from the following formulas:



wherein  $R_I$  is selected from the group consisting of straight and branched alkyls of from 1 to about 8 carbon atoms, benzyl, phenyl, and alkoxy groups and such groups contain-

ing none, one or more than one such substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group consisting of hydrogen, halogens and alkoxy, phenyl and carbonamido groups,  $-COOR_V$  and  $-NHCOOR_V$  wherein  $R_V$  is selected from substituted and unsubstituted alkyl and aryl groups.

The 4-aryloxy group of the invention may function as a timing group and may typically have one of the formulas:



wherein  $m$  is the inhibitor moiety,  $Z'$  is an electron withdrawing group such as nitro, cyano, alkylsulfonyl; sulfamoyl ( $-SO_2NR_2$ ); and sulfonamido ( $-NRSO_2R$ ) groups;  $R_{VI}$  is an alkyl or phenyl group;  $R_{VII}$  is hydrogen or an alkyl group; TIME is a timing group;  $n$  is 0, 1, or 2; and  $p$  is 0 or 1. The oxygen atom is bonded to the 4-position of the 1-arylpolyazol-5-one coupler.

The 4-aryloxy group of the invention which provides a timed release of the inhibitor and the optional timing group (s) which produce(es) the further time-delayed release of the inhibitor group include those such as groups utilizing the cleavage reaction of a hemiacetal (U.S. Pat. No. 4,146,396, Japanese Applications 60-249148; 60-249149); groups using an intramolecular nucleophilic substitution reaction (U.S. Pat. No. 4,248,962); groups utilizing an electron transfer reaction along a conjugated system (U.S. Pat. Nos. 4,409,323; 4,421,845; Japanese Applications 57-188035; 58-98728; 58-209736; 58-209738) groups utilizing ester hydrolysis (German Patent Application (OLS) No. 2,626,315); groups utilizing the cleavage of imino ketals (U.S. Pat. No. 4,546,073); groups that function as a coupler or reducing agent after the coupler reaction (U.S. Pat. Nos. 4,438,193; 4,618,571) and groups that combine the features described above.

It is within the scope of the invention that the coupler of the invention be provided in polymeric form. Thus the coupler may be part of a repeating unit of a polymer. For example, the coupler may be provided via the formula:



where  $Z$  is an aromatic group  $Ar^3Q(n)$  having  $n$  substituents  $Q$ ; where  $n$  is 0 to 5 and the substituent  $Q_1$  is represented by the group:

**5**

where:

& denotes the point of attachment of  $Q_1$  to the  $Ar^3$  ring;  
 k is the number of repeating ethylene units;

$A^1$  represents a hydrogen atom or a lower alkyl group having 1 to 5 carbon atoms;

$A^2$  represents phenylene,  $—COO—$  or  $—CONH—$ ;

$A^3$  represents an alkylene group such as  $—(CH_2)_n—$  where  $n=1$  to 10; or arylene such as o-arylene group, m-arylene group, or p-arylene group;

**6**

$A^4$  represents  $—O—$ ,  $—S—$ ,  $—N(R)C(O)—$ ,  $—C(O)N(R)—$ ,  $—OSO_2—$ ,  $—SO_2—$ ,  $—C(O)O—$ ,  $—OC(O)—$ ,  $—N(R)SO_2—$ , and  $—SO_2N(R)—$  where each R is independently hydrogen or a substituent; and

5 h, i, and j are each 0 or 1 but not all are 0.  
 The coupler can also be a copolymer with at least one repeating unit which is not capable of forming color with oxidized color developing agent.

10 The invention also encompasses a process for forming an image in the described element by contacting an element which has been exposed to light with a color developing chemical,

15 Coupler compounds in accordance with the invention for which Z is  $Ar^3Q(n)$  are exemplified by the following with the corresponding values for the sum of the Hammett (c) constant values for the substituents Q in the  $Ar^3$  ring,  $\Sigma\sigma(Q)$ , and for the P substituents in the  $Ar^4$  ring,  $\Sigma\sigma(P)$ , as shown below. For couplers with Z=alkyl group, only the values of  $\Sigma\sigma(P)$  are listed:

| COUPLER | FORMULA | $\Sigma\sigma(Q)$ | $\Sigma\sigma(P)$ |
|---------|---------|-------------------|-------------------|
| M-1     |         | 0.34              | 0.78              |
| M-2     |         | 0.06              | 0.66              |
| M-3     |         | 0.12              | 0.78              |

-continued

| COUPLER | FORMULA | $\Sigma\sigma(Q)$ | $\Sigma\sigma(P)$ |
|---------|---------|-------------------|-------------------|
| M-4     |         | 0.37              | 0.62              |
| M-5     |         | 0.37              | 0.78              |
| M-6     |         | 0.23              | 0.54              |
| M-7     |         | 0.23              | 0.78              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-8     |    | 0.23              | 0.78              |
| M-9     |   | 0.78              | 0.78              |
| M-10    |  | 0.12              | 0.78              |
| M-11    |  | 0.06              | 0.78              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-12    |    | 0.06              | 0.78              |
| M-13    |   | 0.54              | 0.78              |
| M-14    |  | 0.51              | 0.78              |
| M-15    |  | 0.23              | 0.78              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-16    |    | 0.23              | 0.78              |
| M-17    |   | 0.23              | 0.78              |
| M-18    |  | 0.23              | 0.78              |
| M-19    |  | 0.23              | 0.78              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-20    |    | 0.23              | 0.66              |
| M-21    |   | 0.23              | 0.54              |
| M-22    |  | 0.23              | 0.39              |
| M-23    |  | 0.23              | 0.37              |

-continued

| COUPLER | FORMULA | $\Sigma\sigma(Q)$ | $\Sigma\sigma(P)$ |
|---------|---------|-------------------|-------------------|
| M-24    |         | 0.23              | 0.78              |
| M-25    |         | 0.23              | 0.78              |
| M-26    |         | 0.23              | 0.78              |
| M-27    |         | 0.10              | 0.78              |
| M-28    |         | 0.10              | 0.78              |

-continued

| COUPLER | FORMULA | $\Sigma\sigma(Q)$ | $\Sigma\sigma(P)$ |
|---------|---------|-------------------|-------------------|
| M-29    |         | 0.39              | 0.78              |
| M-30    |         | 0.20              | 0.78              |
| M-31    |         | 0.20              | 0.78              |
| M-32    |         | 0.72              | 0.78              |

-continued

| COUPLER | FORMULA | $\Sigma\sigma(Q)$ | $\Sigma\sigma(P)$ |
|---------|---------|-------------------|-------------------|
| M-33    |         | 0.68              | 0.37              |
| M-34    |         | 0.21              | 0.68              |
| M-35    |         | 0.73              | 0.68              |
| M-36    |         | 0.23              | 0.78              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-37    |    | 0.53              | 0.46              |
| M-38    |    | 0.60              | 0.72              |
| M-39    |   | 0.06              | 0.51              |
| M-40    |  | 0.37              | 0.50              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-41    |    | 0.44              | 0.78              |
| M-42    |   | 0.41              | 0.78              |
| M-43    |  | 0.56              | 3.28              |
| M-44    |  | 0.21              | 0.78              |

-continued

| COUPLER | FORMULA | $\Sigma\sigma(Q)$ | $\Sigma\sigma(P)$ |
|---------|---------|-------------------|-------------------|
| M-45    |         | 0.23              | 0.23              |
| M-46    |         | 0.23              | 0.78              |
| M-47    |         | 0.23              | 0.78              |
| M-48    |         | —                 | 0.78              |

-continued

| COUPLER | FORMULA | $\Sigma\sigma(Q)$ | $\Sigma\sigma(P)$ |
|---------|---------|-------------------|-------------------|
| M-49    |         | —                 | 0.78              |
| M-50    |         | 0.00              | 0.00              |
| M-51    |         | 0.00              | 0.23              |
| M-52    |         | 0.23              | 0.00              |

-continued

| COUPLER | FORMULA                                                                             | $\Sigma\sigma(Q)$ | $\Sigma\sigma(P)$ |
|---------|-------------------------------------------------------------------------------------|-------------------|-------------------|
| M-53    |    | —                 | 0.78              |
| M-54    |   | —                 | 0.23              |
| M-55    |  | —                 | 0.00              |
| M-56    |  | —                 | 0.23              |

-continued

| COUPLER | FORMULA | $\Sigma\sigma(Q)$ | $\Sigma\sigma(P)$ |
|---------|---------|-------------------|-------------------|
| M-57    |         | —                 | 0.00              |
| M-58    |         |                   |                   |
| M-59    |         |                   |                   |

Unless otherwise specifically stated, use of the term "substituted" or "substituent" means any group or atom other than hydrogen. Additionally, when the term "group" is used, it means that when a substituent group contains a substitutable hydrogen, it is also intended to encompass not only the substituent's unsubstituted form, but also its form further substituted with any substituent group or groups as herein mentioned, so long as the substituent does not destroy properties necessary for photographic utility. Suitably, a

60 substituent group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight 65 or branched chain or cyclic alkyl, such as methyl, trifluoromethyl, ethyl, t-butyl, 3-(2,4-di-t-pentylphenoxy) propyl, and tetradecyl; alkenyl, such as ethylene, 2-butene;

35

alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-t-pentylphenoxy)acetamido, alpha-(2,4-di-t-pentylphenoxy)butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, 15 ethoxycarbonylamino, phenoxy carbonylarnino, benzyloxy carbonylamino, hexadecyloxy carbonylamino, 2,4-di-t-butylphenoxy carbonylamino, phenylcarbonylamino, 2,5-(di-t-pentylphenyl)carbonylamino, p-dodecyl-phenylcarbonylamino, 20 p-tolylcarbonylamino, N-methylureido, N,N-dimethylureido, N-methyl-N-dodecylureido, N-hexadecylureido, N,N-dioctadecylureido, N,N-diocetyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as a 25 methylsulfonamido, benzenesulfonamido, p-tolylsulfonamido, p-dodecylbenzenesulfonamido, N-methyltetradecylsulfonamido, N,N-dipropylsulfamoyl, sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diocetylcarbamoyl; acyl, such as acetyl, (2,4-di-t-aminophenoxy)acetyl, phenoxy carbonyl, p-dodecyloxyphenoxy carbonyl methoxycarbonyl, 30 butoxycarbonyl, tetradecyloxy carbonyl, ethoxycarbonyl, benzyloxy carbonyl, 3-pentadecyloxy carbonyl, and dodecyloxy carbonyl; sulfonyl, such as methoxysulfonyl, 35 octyloxy sulfonyl, tetradecyloxy sulfonyl, 2-ethylhexyloxy sulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; 40 sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxyloxy, benzoxyloxy, octadecanoyloxy, 45 p-dodecylamidobenzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1-(N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, 50 a heterocyclic oxy group or a heterocyclic thio group, each of which may be substituted and which contain a 3 to 7

36

membered heterocyclic ring composed of carbon atoms and at least one hetero atom selected from the group consisting of oxygen, nitrogen and sulfur, such as 2-furyl, 2-thienyl, 5 2-benzimidazolyl or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. When a molecule may have two or more substituents, the substituents may be joined together to form a ring such as a fused ring unless otherwise provided. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. Typically, the invention materials are incorporated in a melt and coated as a layer described herein on a support to form 25 part of a photographic element. When the term "associated" is employed, it signifies that a reactive compound is in or adjacent to a specified layer where, during processing, it is capable of reacting with other components.

To control the migration of various components, it may be 30 desirable to include a high molecular weight hydrophobe or "ballast" group in coupler molecules. Representative ballast groups include substituted or unsubstituted alkyl or aryl groups containing 8 to 48 carbon atoms. Representative substituents on such groups include alkyl, aryl, alkoxy, 35 aryloxy, alkylthio, hydroxy, halogen, alkoxy carbonyl, arylox carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can 40 also be further substituted.

The photographic elements can be single color elements or multicolor elements. Multicolor elements contain image 45 dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the 50 three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

If desired, the photographic element can be used in conjunction with an applied magnetic layer as described in 65 *Research Disclosure*, November 1992, Item 34390 published by Kenneth Mason Publications, Ltd., Dudley Annex,

12a North Street, Emsworth, Hampshire P010 7DQ, ENGLAND, and as described in Hatsumi Kyoukai Koukai Gihou No. 94-6023, published Mar. 15, 1994, available from the Japanese Patent Office, the contents of which are incorporated herein by reference. When it is desired to employ the inventive materials in a small format film, *Research Disclosure*, June 1994, Item 36230, provides suitable embodiments.

In the following discussion of suitable materials for use in the emulsions and elements of this invention, reference will be made to *Research Disclosure*, September 1996, Item 38957, available as described above, which is referred to herein by the term "Research Disclosure". The contents of the Research Disclosure, including the patents and publications referenced therein, are incorporated herein by reference, and the Sections hereafter referred to are Sections of the Research Disclosure.

Except as provided, the silver halide emulsion containing elements employed in this invention can be either negative-working or positive-working as indicated by the type of processing instructions (i.e. color negative, reversal, or direct positive processing) provided with the element. Suitable emulsions and their preparation as well as methods of chemical and spectral sensitization are described in Sections I through V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI through VIII. Color materials are described in Sections X through XIII. Suitable methods for incorporating couplers and dyes, including dispersions in organic solvents, are described in Section X(E). Scan facilitating is described in Section XIV. Supports, exposure, development systems, and processing methods and agents are described in Sections XV to XX. The information contained in the September 1994 *Research Disclosure*, Item No. 36544 referenced above, is updated in the September 1996 *Research Disclosure*, Item No. 38957. Certain desirable photographic elements and processing steps, including those useful in conjunction with color reflective prints, are described in *Research Disclosure*, Item 37038, February 1995.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocycl, sulfonamido, mercaptotetrazole, benzothiazole, mercaptopropionic acid, phosphonyloxy, arylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in UK Patents and published application Nos. 1,466,728, 1,531,927, 1,533,039, 2,006, 755A and 2,017,704A, the disclosures of which are incorporated herein by reference.

Image dye-forming couplers may be included in the element such as couplers that form cyan dyes upon reaction with oxidized color developing agents which are described in such representative patents and publications as:

- 5 "Farbkuppler-eine Literature Ubersicht," published in Agfa Mitteilungen, Band III, pp. 156-175 (1961) as well as in U.S. Pat. Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 10 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 15 5,071,737; 5,075,207; 5,091,297; 5,094,938; 5,104,783; 5,178,993; 5,813,729; 5,187,057; 5,192,651; 5,200,305; 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638; 20 5,382,502; 5,384,236; 5,397,691; 5,415,990; 5,434,034; 5,441,863; EPO 0 246 616; EPO 0 250 201; EPO 0 271 323; EPO 0 295 632; EPO 0 307 927; EPO 0 333 185; EPO 0 378 898; EPO 0 389 817; EPO 0 487 111; EPO 0 488 248; EPO 0 539 034; EPO 0 545 300; EPO 0 556 700; EPO 0 556 777; 25 5,402,693; German OLS 3,624,777. and German OLS 3,823,049. Typically such couplers are phenols, naphthols, or pyrazoloazoles.

Couplers that form magenta dyes upon reaction with oxidized color developing agent are described in such representative patents and publications as: "Farbkuppler-eine Literature Ubersicht," published in Agfa Mitteilungen, Band III, pp. 126-156 (1961) as well as U.S. Pat. Nos. 2,311,082 and 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 40 4,914,013; 4,921,968; 4,929,540; 4,933,465; 4,942,116; 4,942,117; 4,942,118; 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 45 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EPO 0 257 854; EPO 0 284 240; EPO 0 341 204; EPO 347,235; EPO 365,252; EPO 0 422 595; EPO 0 428 899; EPO 0 428 902; EPO 0459331; EPO 0467327; EPO 0476949; EPO 0487081; EPO 0489333; EPO 0512304; EPO 0515

128; EPO 0534703; EPO 0554778; EPO 0558 145; EPO 0 571 959; EPO 0 583 832; EPO 0 583 834; EPO 0 584 793; EPO 0 602 748; EPO 0 602 749; EPO 0 605 918; EPO 0 622 672; EPO 0 622 673; EPO 0 629 912; EPO 0 646 841, EPO 0 656 561; EPO 0 660 177; EPO 0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265; and German OLS 40 08 067. Typically such couplers are pyrazolones, pyrazoloazoles, or pyrazolobenzimidazoles that form magenta dyes upon reaction with oxidized color developing agents.

Couplers that form yellow dyes upon reaction with oxidized color developing agent are described in such repre-

sentative patents and publications as: "Farbkuppler-eine Literature Ubersicht," published in Agfa Mitteilungen; Band III; pp. 112-126 (1961); as well as U.S. Pat. Nos. 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773; 5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474; 5,405,737; 5,411,848; 5,427,898; EPO 0 327 976; EPO 0 296 793; EPO 0 365 282; EPO 0 379 309; EPO 0 415 375; EPO 0 437 818; EPO 0 447 969; EPO 0 542 463; EPO 0 568 037; EPO 0 568 196; EPO 0 568 777; EPO 0 570 006; EPO 0 573 761; EPO 0 608 956; EPO 0 608 957; and EPO 0 628 865. Such couplers are typically open chain ketomethylene compounds.

Couplers that form colorless products upon reaction with oxidized color developing agent are described in such representative patents as: UK. 861,138; U.S. Pat. Nos. 3,632,345; 3,928,041; 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No. 2,644,194 and German OLS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628, 5,151,343, and 5,234,800.

It may be useful to use a combination of couplers any of which may contain known ballasts or coupling-off groups such as those described in U.S. Pat. Nos. 4,301,235; 4,853,319 and 4,351,897. The coupler may contain solubilizing groups such as described in U.S. Pat. No. 4,482,629. The coupler may also be used in association with "wrong" colored couplers (e.g. to adjust levels of interlayer correction) and, in color negative applications, with masking couplers such as those described in EP 213,490; Japanese Published Application 58-172,647; U.S. Pat. Nos. 2,983,608; 4,070,191; and 4,273,861; German Applications DE 2,706,117 and DE 2,643,965; UK. Patent 1,530,272; and Japanese Application 58-113935. The masking couplers may be shifted or blocked, if desired.

Useful coated levels of the couplers of this invention range from about 0.010 to 2.15 g/m<sup>2</sup> or more typically 0.03 to 1.50 g/m<sup>2</sup>. Typically, couplers are incorporated in a silver halide emulsion layer in a mole ratio to silver of 0.05 to 1.0 and generally 0.1 to 0.5. The couplers of this invention are usually utilized by dissolving them in high-boiling coupler solvents and then dispersing the organic coupler plus coupler solvent mixtures as small particles in aqueous solutions of gelatin and surfactant (via milling or homogenization). Removable auxiliary organic solvents such as ethyl acetate or cyclohexanone may also be used in the preparation of such dispersions to facilitate the dissolution of the coupler in the organic phase. Coupler solvents useful for the practice of

this invention include aryl phosphates (e.g. trityl phosphate), alkyl phosphates (e.g. trioctyl phosphate), mixed aryl alkyl phosphates (e.g. diphenyl 2-ethylhexyl phosphate), aryl, alkyl or mixed aryl-alkyl phosphonates, phosphine oxides (e.g. trioctylphosphine oxide), esters of aromatic acids (e.g. dibutyl phthalate, octyl benzoate, or benzyl salicylate), esters of aliphatic acids (e.g. acetyl tributyl citrate, tripentyl citrate, or dibutyl sebacate), alcohols (e.g. 2-hexyl-1-decanol), phenols (e.g. p-dodecylphenol), carbonamides (e.g. N,N-dibutyldecanamide or N-butylacetanilide), sulfoxides (e.g. bis(2-ethylhexyl) sulfoxide), sulfonamides (e.g. N,N-dibutyl-p-toluenesulfonamide) or hydrocarbons (e.g. dodecylbenzene). Additional coupler solvents and auxiliary solvents are noted in Research Disclosure, December 1989, Item 308119, p. 993. Useful coupler: coupler solvent weight ratios range from about 1:0.1 to 1:8.0 with 1:0.2 to 1:4.0 being preferred. Dispersions using no permanent coupler solvent are sometimes employed.

The invention materials may be used in association with materials that release Photographically Useful Groups (PUGS) that accelerate or otherwise modify the processing steps e.g. of bleaching or fixing to improve the quality of the image. Bleach accelerator releasing couplers such as those

described in EP 193,389; EP 301,477; U.S. Pat. Nos. 4,163,669; 4,865,956; and 4,923,784, may be useful. Also contemplated is use of the compositions in association with nucleating agents, development accelerators or their precursors (UK Patent 2,097,140; UK. Patent 2,131,188); electron transfer agents (U.S. Pat. Nos. 4,859,578; 4,912,025); anti-fogging and anti color-mixing agents such as derivatives of hydroquinones, amminophenols, amines, gallic acid; catechol; ascorbic acid; hydrazides; sulfonamidophenols; and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. Nos. 4,420,556; and 4,543,323.) Also, the compositions may be blocked or coated in protected form as described, for example, in Japanese Application 61/258,249 or U.S. Pat. No. 5,019,492.

The invention materials may further be used in combination with image-modifying compounds that release PUGS such as "Developer Inhibitor-Releasing" compounds (DIR's). DIR's useful in conjunction with the compositions of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography,"

C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptotriazoles, mercaptooxadiazoles, mercaptodiazoles, mercaptooxathiazoles, tellurotetrazoles or benzisodiazoles. In a preferred embodiment, the inhibitor moiety or group is selected from the following formulas:



wherein  $R_1$  is selected from the group consisting of straight and branched alkyls of from 1 to about 8 carbon atoms, benzyl, phenyl, and alkoxy groups and such groups containing none, one or more than one such substituent;  $R_2$  is selected from  $R_1$  and  $-SR_1$ ;  $R_3$  is a straight or branched alkyl group of from 1 to about 5 carbon atoms and  $m$  is from 1 to 3; and  $R_4$  is selected from the group consisting of hydrogen, halogens and alkoxy, phenyl and carbonamido groups,  $-COOR_V$  and  $-NHCOR_V$  wherein  $R_V$  is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers).

A compound such as a coupler may release a PUG directly upon reaction of the compound during processing, or indirectly through a timing or linking group. A timing group produces the time-delayed release of the PUG such groups using an intramolecular nucleophilic substitution reaction (U.S. Pat. No. 4,248,962); groups utilizing an electron transfer reaction along a conjugated system (U.S. Pat. Nos. 4,409,323; 4,421,845; 4,861,701, Japanese Applications 57-188035; 58-98728; 58-209736; 58-209738); groups that function as a coupler or reducing agent after the coupler reaction (U.S. Pat. Nos. 4,438,193; 4,618,571) and groups that combine the features described above. It is typical that the timing group is of one of the formulas:



wherein IN is the inhibitor moiety,  $R_7$  is selected from the group consisting of nitro, cyano, alkylsulfonyl; sulfamoyl; and sulfonamido groups;  $a$  is 0 or 1; and  $R_7$  is selected from the group consisting of substituted and unsubstituted alkyl and phenyl groups. The oxygen atom of each timing group is bonded to the coupling-off position of the respective coupler moiety of the DIAR.

The timing or linking groups may also function by electron transfer down an unconjugated chain. Linking groups are known in the art under various names. Often they have been referred to as groups capable of utilizing a hemiacetal or iminoketal cleavage reaction or as groups capable of utilizing a cleavage reaction due to ester hydrolysis such as U.S. Pat. No. 4,546,073. This electron transfer down an unconjugated chain typically results in a relatively fast decomposition and the production of carbon dioxide, formaldehyde, or other low molecular weight by-products. The groups are exemplified in EP 464,612, EP 523,451, U.S. Pat. No. 4,146,396, Japanese Kokai 60-249148 and 60-249149.

Suitable developer inhibitor-releasing couplers for use in the present invention include, but are not limited to, the following:



6,156,490

**43**

-continued



D2



D3



D4



D5

**44**

-continued

D6



D7



D8



5

10

15

20

25

30

35

40

45

50

55

60

**45**

-continued



D9

**46**

-continued



D12



D10



D11

20 It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire P0101 7DQ, England, incorporated herein by reference. Materials of the invention may be coated on pH adjusted support as described in U.S. Pat. No. 4,917,994; on a support with reduced oxygen permeability (EP 553,339); with epoxy 25 solvents (EP 164,961); with nickel complex stabilizers (U.S. Pat. Nos. 4,346,165; 4,540,653 and 4,906,559 for example); with ballasted chelating agents such as those in U.S. Pat. No. 4,994,359 to reduce sensitivity to polyvalent cations such as 30 calcium; and with stain reducing compounds such as described in U.S. Pat. No. 5,068,171. Other compounds useful in combination with the invention are disclosed in Japanese Published Applications described in Derwent 35 Abstracts having accession numbers as follows: 90-072,629, 90-072,630; 90-072,631; 90-072,632; 90-072,633; 90-072, 634; 90-077,822; 90-078,229; 90-078,230; 90-079,336; 90-079,337; 90-079,338; 90-079,690; 90-079,691; 90-080, 40 487; 90-080,488; 90-080,489; 90-080,490; 90-080,491; 90-080,492; 90-080,494; 90-085,928; 90-086,669; 90-086, 45 670; 90-087,360; 90-087,361; 90-087,362; 90-087,363; 90-087,364; 90-088,097; 90-093,662; 90-093,663; 90-093, 50 664; 90-093,665; 90-093,666; 90-093,668; 90-094,055; 90-094,056; 90-103,409; 83-62,586; 83-09,959.

Conventional radiation-sensitive silver halide emulsions can be employed in the practice of this invention. Such 55 emulsions are illustrated by *Research Disclosure*, Item 38755, September 1996, 1. Emulsion grains and their preparation.

Especially useful in this invention are tabular grain silver 60 halide emulsions. Tabular grains are those having two parallel major crystal faces and having an aspect ratio of at least 2. The term "aspect ratio" is the ratio of the equivalent circular diameter (ECD) of a grain major face divided by its thickness (t). Tabular grain emulsions are those in which the 65

tabular grains account for at least 50 percent (preferably at least 70 percent and optimally at least 90 percent) of the total grain projected area. Preferred tabular grain emulsions are those in which the average thickness of the tabular grains is less than 0.3 micrometer (preferably thin—that is, less than 0.2 micrometer and most preferably ultrathin—that is, less than 0.07 micrometer). The major faces of the tabular grains can lie in either {111} or {100} crystal planes. The mean ECD of tabular grain emulsions rarely exceeds 10 micrometers and more typically is less than 5 micrometers.

In their most widely used form tabular grain emulsions are high bromide {111} tabular grain emulsions. Such emulsions are illustrated by Kofron et al U.S. Pat. No. 4,439,520, Wilgus et al U.S. Pat. No. 4,434,226, Solberg et al U.S. Pat. No. 4,433,048, Maskasky U.S. Pat. Nos. 4,435, 501, 4,463,087 and 4,173,320, Daubendiek et al U.S. Pat. Nos. 4,414,310 and 4,914,014, Sowinski et al U.S. Pat. No. 4,656,122, Pigglin et al U.S. Pat. Nos. 5,061,616 and 5,061, 609, Tsaur et al U.S. Pat. Nos. 5,147,771, '772, '773, 5,171,659 and 5,252,453, Black et al 5,219,720 and 5,334, 495, Delton U.S. Pat. Nos. 5,310,644, 5,372,927 and 5,460, 934, Wen U.S. Pat. No. 5,470,698, Fenton et al U.S. Pat. No. 5,476,760, Eshelman et al U.S. Pat. Nos. 5,612,175 and 5,614,359, and Irving et al U.S. Pat. No. 5,667,954.

Ultrathin high bromide {111} tabular grain emulsions are illustrated by Daubendiek et al U.S. Pat. Nos. 4,672,027, 4,693,964, 5,494,789, 5,503,971 and 5,576,168, Antoniades et al U.S. Pat. No. 5,250,403, Olm et al U.S. Pat. No. 5,503,970, Deaton et al U.S. Pat. No. 5,582,965, and Maskasky U.S. Pat. No. 5,667,955.

High bromide {100} tabular grain emulsions are illustrated by Mignot U.S. Pat. Nos. 4,386,156 and 5,386,156.

High chloride {111} tabular grain emulsions are illustrated by Wey U.S. Pat. No. 4,399,215, Wey et al U.S. Pat. No. 4,414,306, Maskasky U.S. Pat. Nos. 4,400,463, 4,713, 323, 5,061,617, 5,178,997, 5,183,732, 5,185,239, 5,399,478 and 5,411,852, and Maskasky et al U.S. Pat. Nos. 5,176,992 and 5,178,998. Ultrathin high chloride {111} tabular grain emulsions are illustrated by Maskasky U.S. Pat. Nos. 5,271, 858 and 5,389,509.

High chloride {100} tabular grain emulsions are illustrated by Maskasky U.S. Pat. Nos. 5,264,337, 5,292,632, 5,275,930 and 5,399,477, House et al U.S. Pat. No. 5,320, 938, Brust et al U.S. Pat. No. 5,314,798, Szajewski et al U.S. Pat. No. 5,356,764, Chang et al U.S. Pat. Nos. 5,413,904 and 5,663,041, Oyamada U.S. Pat. No. 5,593,821, Yamashita et al U.S. Pat. Nos. 5,641,620 and 5,652,088, Saitou et al U.S. Pat. No. 5,652,089, and Oyamada et al U.S. Pat. No. 5,665,530. Ultrathin high chloride {100} tabular grain emulsions can be prepared by nucleation in the presence of iodide, following the teaching of House et al and Chang et al, cited above.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent. Tabular grain emulsions of the latter type are illustrated by Evans et al. U.S. Pat. No. 4,504,570.

Photographic elements can be exposed to actinic radiation, typically in the visible region of the spectrum, to form a latent image and can then be processed to form a

visible dye image. Processing to form a visible dye image includes the step of contacting the element with a color developing agent to reduce developable silver halide and oxidize the color developing agent. Oxidized color developing agent in turn reacts with the coupler to yield a dye. If desired "Redox Amplification" as described in Research Disclosure XVIIIB(5) may be used.

With negative-working silver halide, the processing step described above provides a negative image. One type of such element, referred to as a color negative film, is designed for image capture. Speed (the sensitivity of the element to low light conditions) is usually critical to obtaining sufficient image in such elements. Such elements are typically silver bromoiodide emulsions coated on a transparent support and are sold packaged with instructions to process in known color negative processes such as the Kodak C-41 process as described in The British Journal of Photography Annual of 1988, pages 191-198. If a color negative film element is to be subsequently employed to generate a viewable projection print as for a motion picture, a process such as the Kodak ECN-2 process described in the H-24 Manual available from Eastman Kodak Co. may be employed to provide the color negative image on a transparent support. Color negative development times are typically 3' 15" or less and desirably 90 or even 60 seconds or less.

The photographic element of the invention can be incorporated into exposure structures intended for repeated use or exposure structures intended for limited use, variously referred to by names such as "single use cameras", "lens with film", or "photosensitive material package units".

Another type of color negative element is a color print. Such an element is designed to receive an image optically printed from an image capture color negative element. A color print element may be provided on a reflective support for reflective viewing (e.g. a snap shot) or on a transparent support for projection viewing as in a motion picture. Elements destined for color reflection prints are provided on a reflective support, typically paper, employ silver chloride emulsions, and may be optically printed using the so-called negative-positive process where the element is exposed to light through a color negative film which has been processed as described above. The element is sold packaged with instructions to process using a color negative optical printing process, for example the Kodak RA-4 process, as generally described in PCT WO 87/04534 or U.S. Pat. No. 4,975,357, to form a positive image. Color projection prints may be processed, for example, in accordance with the Kodak ECP-2 process as described in the H-24 Manual. Color print development times are typically 90 seconds or less and desirably 45 or even 30 seconds or less.

A reversal element is capable of forming a positive image without optical printing. To provide a positive (or reversal) image, the color development step is preceded by development with a non-chromogenic developing agent to develop exposed silver halide, but not form dye, and followed by uniformly fogging the element to render unexposed silver halide developable. Such reversal elements are typically sold packaged with instructions to process using a color reversal process such as the Kodak E-6 process as described in The British Journal of Photography Annual of 1988, page 194. Alternatively, a direct positive emulsion can be employed to obtain a positive image.

The above elements are typically sold with instructions to process using the appropriate method such as the mentioned color negative (Kodak C-41), color print (Kodak RA-4), or reversal (Kodak E-6) process.

Preferred color developing agents are *p*-phenylenediamines such as:

49

4-amino-N,N-diethylaniline hydrochloride,  
 4-amino-3-methyl-N,N-diethylaniline hydrochloride,  
 4-amino-3-methyl-N-ethyl-N-(2-methanesulfonamidoethyl)aniline sesquisulfate hydrate,

50

The entire contents of the patents and other publications referred to in this specification are incorporated herein by reference.

### Synthesis Example: Compound M-7



### 4-amino-3-methyl-N-ethyl-N-(2-hydroxyethyl)aniline sulfate,

4-amino-3-(2-methanesulfonamidoethyl)-N,N-diethylaniline hydrochloride, and

4-amino-N-ethyl-N-(2-methoxyethyl)-m-toluidine di-p-toluene sulfonic acid.

Development is usually followed by the conventional 65 steps of bleaching, fixing, or bleach-fixing, to remove silver or silver halide, washing, and drying.

## Preparation of p-Nitrophenoxyacetophenone 2.

Solid potassium carbonate (16.59 g, 120 mmol) was added to a solution of 1 (23.35 g, 100 mmol) and p-nitrophenol (15.30 g, 110 mmol) in 250 mL of N,N-dimethylformamide. The resulting mixture was stirred at room temperature under nitrogen for 1 h and poured into 1000 mL of water giving a solid. After stirring for 2 h the solid was filtered off, washed with water (7×200 mL),

hexanes (3×50 mL), and dried in vacuo. The yield of 2 was 28.54 g (98 mmol, 98%).

Preparation of the Enamine 3.

p-Toluenesulfonic acid monohydrate (50 mg) was added to a solution of 2 (2.92 g, 10 mmol) and pyrrolidine (2.5 mL; 36 mmol) in 25 mL of toluene. The mixture was refluxed under nitrogen using a Dean-Stark trap for 3 h, cooled to room temperature and washed with water (3×15 mL). The solvent was distilled off in vacuo leaving 3 as a dark-red oil.

Preparation of the  $\beta$ -Ketoanilide 4.

Solid p-nitrophenylisocyanate (1.64 g, 10 mmol) was added to the solution of 3 (ca. 10 mmol) in 30 mL of toluene and the resulting solution was refluxed for 1 h. The solvent was distilled off, the residue taken up in methanol (30 mL), and the mixture refluxed with concentrated hydrochloric acid (1 mL) for 20 min giving a solid. After cooling to room temperature the mixture was filtered, the solid washed with methanol (2×10 mL) and dried in vacuo. The yield of 4 was 3.39 g (7.4 mmol, 74%).

Preparation of M-7.

Solid ballasted phenylhydrazine hydrochloride 5 (2.77 g, 6 mmol) was added in small portions over a period of 45 min to a refluxing solution of 4 (2.28 g, 5 mmol) in propyl acetate (50 mL). Following the addition the solution was refluxed for 1 h. After cooling to room temperature the solution was diluted with propyl acetate and worked up with diluted hydrochloric acid, washed with water, dried over magnesium sulfate and concentrated to an oil. The crude product was purified by column chromatography on silica gel giving an oil which crystallized when stirred with hexanes (10 mL) for 24 h. The yield of M-7 was 1.40 g (1.9 mmol, 39%); m.p. 160°–162° C., M<sup>+</sup>724.

Photographic Examples

The comparative couplers and inventive couplers used for the photographic examples were dispersed and coated with the high-boiling solvent trityl phosphate (S-1, mixed isomers). The dispersions were prepared by adding an oil phase containing a 1:1:3 weight ratio of coupler:trityl phosphate:ethyl acetate to an aqueous phase containing gelatin and the dispersing agent ALKANOL XC (Dupont) in a 10:1 weight ratio. Each of the resulting mixtures was passed through a colloid mill to disperse the coupler-containing oil phase in the aqueous phase as small particles. The resulting dispersions contained 2% by weight of coupler and 6% by weight of gelatin.

Sufficient coupler dispersion to yield a laydown of 0.646 mmol/sq.m was mixed with a silver iodobromide emulsion and additional gelatin and coated on cellulose acetate butyrate support. On coating, the ethyl acetate auxiliary solvent in the dispersion evaporates. The layer containing coupler and silver halide was overcoated with a layer containing gelatin and the hardener bis (vinylsulfonylmethyl) ether. The coating structure is shown in Table I with laydowns in g/sq m given in parenthesis (except where noted).

TABLE I

| Overcoat:                                      |
|------------------------------------------------|
| Gelatin (5.38)                                 |
| Bis(vinylsulfonylmethyl)ether Hardener (0.161) |
| Gelatin (2.69)                                 |
| Magenta dye-forming coupler (0.646 mmol/sq.m)  |

TABLE I-continued

| Overcoat:                                                                                                                                                           |
|---------------------------------------------------------------------------------------------------------------------------------------------------------------------|
| & Tritolyt phosphate(S-1) at equal weight to coupler<br>Ag as a 0.46 $\mu$ m silver bromoiodide (6.4% iodide) emulsion (1.61)<br>cellulose acetate butyrate support |

After hardening, samples of each of the films were exposed through a step tablet on a 1B sensitometer and processed using the KODAK FLEXICOLOR C-41 color negative procedure A, or modified procedure B, described in Table II. The developer in procedure B contains 4.0 g/l citrazinic acid (CZA) which competes with the in-film comparative and inventive couplers for oxidized developer, Measurements of status M green density vs. exposure were made for each processed film strip, and photographic contrast (gamma,  $\gamma$ ) was determined from the slopes of such plots.

TABLE II

| C-41 Processing Solutions and Conditions                                              |                 |               |
|---------------------------------------------------------------------------------------|-----------------|---------------|
| Solution                                                                              | Processing Time | Agitation Gas |
| A) C-41 Developer<br>or<br>B) C-41 Developer plus<br>4.0 g/l Citrazinic<br>Acid (CZA) | 3'15"           | Nitrogen      |
| Stop Bath                                                                             | 30"             | Nitrogen      |
| Bleach                                                                                | 3'              | Air           |
| Wash                                                                                  | 1'              | None          |
| Fix                                                                                   | 4'              | Nitrogen      |
| Wash                                                                                  | 4'              | None          |
| Bath containing<br>wetting agent                                                      | 30"             | None          |
| Processing temperature 100° F.                                                        |                 |               |

The activity of a coupler in film can be related to the resistance of its gamma in processing Procedure A ( $\gamma_{C41}$ ) from being reduced in processing Procedure B ( $\gamma_{CZA}$ ). One way to represent the activity is by the formula:

$$ACT = (\gamma_{CZA}/\gamma_{C41}) \times 100$$

The higher the number, the more active the coupler.

To evaluate the stability of the coupler, film samples were subjected to an accelerated raw stock-keeping test. The test consisted of storage of unexposed, unprocessed samples at 100° C. and 50% relative humidity for 4 weeks. Samples were then exposed and processed in Procedure A. Values of Dmax, the maximum density obtained at high exposure, were compared to the earlier Procedure A processed, unkept films. Dmax values were corrected for Dmin to remove contributions to green density from the support and other coating components. The ratio of the corrected Dmax obtained from an incubated sample relative, to the corrected Dmax of a sample of the same film processed immediately following hardening, is referred to as the Density Ratio (DR).

$$DR = [(D_{max,incubated} - D_{min}) / (D_{max,fresh} - D_{min})] \times 100$$

This ratio is a measure of the raw stock stability of the coupler in the film composition. The higher the number, the more stable the coupler. Many of the couplers were coated in different sets. To reduce variation when comparing sets, CK-1 was coated, processed, and incubated in a like to comparative and inventive couplers and used as an internal check in all keeping tests. Its value for Density Ratio over many experiments was averaged and used to normalize the Density Ratios for the comparative and inventive couplers:  
10



DR(normalized)=[DR(CK-1 average)/DR(CK-1 for set)]xDR(test)  
15

In the following examples, the indicated comparison examples were employed:

| COUPLER | FORMULA | $\Sigma\sigma(Q)$ | $\Sigma\sigma(P)$ |
|---------|---------|-------------------|-------------------|
| C-1     |         | 0.00              | 0.00              |
| C-2     |         | 0.00              | 0.23              |
| C-3     |         | 0.23              | 0.00              |

-continued

| COUPLER | FORMULA | $\Sigma\sigma(Q)$ | $\Sigma\sigma(P)$ |
|---------|---------|-------------------|-------------------|
| C-4     |         | 0.23              | 0.23              |
| C-5     |         | —                 | 0.78              |
| C-6     |         | —                 | 0.78              |

## EXAMPLE 1

Couplers of this invention M-45, M-50, M-51, and M-52, and comparison couplers C-1, C-2, C-3, and C-4 were dispersed and coated as described, and processed in Procedure A and B. In addition, film samples were subjected to an accelerated raw stock keeping test under the conditions indicated, exposed and processed, and normalized Density Ratios determined as described. The inventive couplers all have ortho substituent groups on the 1-nitrogen phenyl whereas the comparative couplers all possess para substituents on the 1-nitrogen phenyl ring. These couplers form sets of similarly substituted couplers in the 4-carbon coupling off group and 3-carbon phenyl position except for the ortho vs. para substitution: C-1 vs. M-50, C-2 vs. M-51, C-3 vs. M-52, and C-4 vs. M-45. Table III shows the results of the tests.

TABLE III

| 55   | Coupler | Type | Density Ratio + Activity Improvements |                   |                                |       |
|------|---------|------|---------------------------------------|-------------------|--------------------------------|-------|
|      |         |      | $\Sigma\sigma(Q)$                     | $\Sigma\sigma(P)$ | Density Ratio(DR) <sup>1</sup> | ACT   |
| C-1  | Comp    | 0.00 | 0.00                                  | 41.2              | 88.8                           | 130.0 |
| C-2  | Comp    | 0.00 | 0.23                                  | 62.0              | 90.8                           | 152.8 |
| C-3  | Comp    | 0.23 | 0.00                                  | 55.6              | 89.5                           | 145.1 |
| C-4  | Comp    | 0.23 | 0.23                                  | 77.8              | 92.8                           | 170.6 |
| M-50 | Inv     | 0.00 | 0.00                                  | 96.1              | 84.5                           | 180.6 |
| M-51 | Inv     | 0.00 | 0.23                                  | 93.5              | 87.3                           | 180.8 |
| M-52 | Inv     | 0.23 | 0.00                                  | 99.2              | 85.1                           | 184.2 |
| M-45 | Inv     | 0.23 | 0.23                                  | 100.0             | 82.3                           | 182.3 |

<sup>1</sup>Keeping results are based on 4 weeks @ 100° F. and are normalized.

Both raw stock stability and coupler activity are important properties of couplers in films. Preferred raw stock keeping is 95 or better, with a value of 85 being acceptable. Preferred coupler activity is 75 or higher, with 70 being acceptable. However, in the absence of at least acceptable raw stock stability, activity is of no value. Therefore, we have found that while both keeping and activity must satisfy at least the acceptable criteria, an important metric is that the sum of activity (ACT) and keeping (DR) be greater than 170 with the density ratio for raw stock stability being at least 85.

It is evident from the sum of normalized Density Ratio values and Activities in Table III that the photographic elements of the invention which contain the specified ortho substituted magenta dye forming couplers show satisfactory values in the sum test, all being greater than 170—in fact being greater than 180. In addition the Density Ratio values all show outstanding stability in the raw stock keeping test, with almost all values being in the preferred range. When viewed in pairs of similarly substituted couplers, the ortho inventive coupler is always superior to the comparative para example. The inventive ortho materials exceed the ACT+DR=170 requirement, and DR exceeds the 85 requirement in all examples. The para comparison couplers failed to produce acceptable results. In the one case that the comparative example, C-4, barely meets the ACT+DR=170 requirement, DR is only 77.8—outside of the DR criteria.

#### EXAMPLE 2

Photographic element samples were prepared and tested in a manner similar to Example 1, except this time the carbon-3 substituent was an alkyl group rather than phenyl group. The coupling-off group was held constant. The inventive couplers all have ortho substituent groups on the 1-nitrogen phenyl whereas the comparative couplers all possess para substituents on the 1-nitrogen phenyl ring. These couplers form sets of similarly substituted couplers in the 4-carbon coupling off group and 3-carbon alkyl position except for the ortho vs. para substitution: Table IV shows the results of testing.

TABLE V

#### MULTILAYER FILM STRUCTURE

|   |                      |                                                                                                                                                                                                                                                                                                                                                                                                                            |
|---|----------------------|----------------------------------------------------------------------------------------------------------------------------------------------------------------------------------------------------------------------------------------------------------------------------------------------------------------------------------------------------------------------------------------------------------------------------|
| 1 | Overcoat & UV Layer: | Matte Bead<br>UV Absorbers Uv-1 (0.108), UV-2 (0.108) & S-1 (0.151)<br>Silver Bromide Lippmann Emulsion (0.215 Ag)<br>Gelatin (1.237)                                                                                                                                                                                                                                                                                      |
| 2 | Fast Yellow Layer:   | Bis(vinylsulfonyl)methane Hardener (1.75% of Total Gelatin)<br>Y-1 (0.237)Yellow Dye-Forming Coupler & S-1 (0.118)<br>IR-1 (0.076) DIR Coupler & S-1 (0.038)<br>B-1 (0.0054) BARC & S-3 (0.0070)<br>Blue Sensitive Silver Iodobromide Emulsion (0.377 Ag), 4.1 mole % Iodide T-Grain (2.9 × 0.12 μm)<br>Blue Sensitive Silver Iodobromide Emulsion (0.108 Ag) 4.1 mole % Iodide T-Grain (1.9 × 0.14 μm)<br>Gelatin (0.807) |
| 3 | Slow Yellow Layer:   | Y-1 (1.076) & S-1 (0.538)<br>IR-1 (0.076) & S-1 (0.038)<br>B-1 (0.022) & S-3 (0.028)<br>CC-1 (0.032) & S-2 (0.064)<br>IR-4 (0.032) & S-2 (0.064)<br>Blue Sensitive Silver Iodobromide Emulsion (0.398 Ag), 4.1 mole % Iodide T-Grain (1.9 × 0.14 μm)                                                                                                                                                                       |

TABLE IV

| Coupler | Type | Density Ratio + Activity Improvements |                   |                                | ACT  | DR + ACT |
|---------|------|---------------------------------------|-------------------|--------------------------------|------|----------|
|         |      | $\Sigma\alpha(Q)$                     | $\Sigma\alpha(P)$ | Density Ratio(DR) <sup>1</sup> |      |          |
| C-5     | Comp | —                                     | 0.78              | 74.4                           | 86.1 | 160.5    |
| C-6     | Comp | —                                     | 0.78              | 61.3                           | 81.4 | 142.7    |
| M-48    | Inv  | —                                     | 0.78              | 100                            | 73.7 | 173.7    |
| M-49    | Inv  | —                                     | 0.78              | 100                            | 81.4 | 181.4    |
| M-53    | Inv  | —                                     | 0.78              | 100                            | 77.0 | 177.0    |

<sup>1</sup>Keeping results are based on 4 weeks @ 100° F. and are normalized.

It is evident from the sum of normalized Density Ratio values and Activities in Table IV that the photographic elements of the invention which contain the specified ortho substituted magenta dye forming couplers show satisfactory values in the sum test, all being greater than 170. In addition the Density Ratio values all show outstanding stability in the raw stock keeping test, with all values being in the preferred range. When viewed in pairs of similarly substituted couplers, the ortho inventive coupler is always superior to the comparative para example (M-48 vs. C-5, M-49 vs. C-6). The inventive ortho materials exceed the ACT+DR=170 requirement, and DR exceeds the 85 requirement in all examples. The para comparison couplers failed to satisfy either criteria.

#### EXAMPLE 3

#### Multilayer Film Structure Comprising a 4-Aryloxyypyrazolone Coupler of This Invention

The multilayer film structure utilized for this example is shown schematically in Table V. Structures of components not provided previously are given immediately following Table V. Component laydowns are provided in units of g/sq m unless otherwise indicated. This composition may also be coated on a support, such as polyethylene naphthalate, containing a magnetic recording layer. The use of the 4-aryloxy-1-arylpypyrazolo-5-one imaging coupler M-52 of this invention provides reduced coupler laydowns useful for layer thinning and improved sharpness. The color negative film described in Table V may be processed using KODAK FLEXICOLOR C-41 chemistry to yield excellent latitude and sharpness.

TABLE V-continued

## MULTILAYER FILM STRUCTURE

|                        |                                                                                                                                                                                                                                                                                                                                                                       |
|------------------------|-----------------------------------------------------------------------------------------------------------------------------------------------------------------------------------------------------------------------------------------------------------------------------------------------------------------------------------------------------------------------|
|                        | Blue Sensitive Silver Iodobromide Emulsion (0.269 Ag), 1.3 mole % Iodide T-Grain (0.54 x 0.08 $\mu\text{m}$ )<br>Blue Sensitive Silver Iodobromide Emulsion (0.247 Ag) 1.5 mole % Iodide T-Grain (0.77 x 0.14 $\mu\text{m}$ )<br>Gelatin (1.872)                                                                                                                      |
| 4 Yellow Filter Layer: | R-1 (0.086) & S-2 (0.139) & ST-2 (0.012)<br>YD-2 Filter Dye (0.054)<br>Gelatin (0.646)                                                                                                                                                                                                                                                                                |
| 5 Fast Magenta Layer   | M-52 (0.062) Inventive Magenta Dye-Forming Coupler & S-1 (0.062)<br>R-2 (0.009)<br>MM-1 (0.054) Masking Coupler & S-1 (0.108)<br>IR-3 (.030) DIR Coupler & S-2 (0.060)<br>B-1 (0.003) & S-3 (0.004)<br>Green Sensitive Silver Iodobromide Emulsion (0.484 Ag), 4.0 mole % Iodide T-Grain (1.60 x 0.12 $\mu\text{m}$ )<br>Gelatin (1.014)                              |
| 6 Mid Magenta Layer:   | M-52 (0.102) & S-1 (0.102)<br>MM-1 (0.118) & S-1 (0.236), R-2 (0.015)<br>IR-2 (0.043) DIR Coupler & S-2 (0.043)<br>Green Sensitive Silver Iodobromide Emulsion (0.247 Ag), 4.0 mole % Iodide T-Grain (1.20 x 0.11 $\mu\text{m}$ )<br>Green Sensitive Silver Iodobromide Emulsion (0.247 Ag) 4.0 mole % Iodide T-Grain (1.00 x 0.12 $\mu\text{m}$ )<br>Gelatin (1.216) |
| 7 Slow Magenta Layer:  | M-52 (0.222) & S-1 (0.222)<br>MM-1 (0.086) & S-1 (0.172)<br>IR-2 (0.011) & S-2 (0.011)<br>Green Sensitive Silver Iodobromide Emulsion (0.344 Ag), 3.5 mole % Iodide T-Grain (0.90 x 0.12 $\mu\text{m}$ )<br>Green Sensitive Silver Iodobromide Emulsion (0.129 Ag), 1.5 mole % Iodide T-Grain (0.50 x 0.08 $\mu\text{m}$ )<br>Gelatin (1.076)                         |
| 8 Interlayer:          | R-1 (0.086) Interlayer Scavenger, S-2 (0.139) & ST-2 (0.012)<br>Gelatin (0.538)                                                                                                                                                                                                                                                                                       |
| 9 Fast Cyan Layer:     | CC-1 (0.183) Cyan Dye-Forming Coupler & S-2 (0.210)<br>CM-1 (0.022) Masking Coupler<br>IR4 (0.027) DIAR Coupler & S-2 (0.054)<br>Red Sensitive Silver Iodobromide Emulsion (0.592 Ag),<br>4.1 mole % Iodide T-Grain (1.7 x 0.12 $\mu\text{m}$ )<br>Gelatin (0.915)                                                                                                    |
| 10 Mid Cyan Layer:     | CC-1 (0.170) & S-2 (0.190)<br>CM-1 (0.032)<br>B-1 (0.008) & S-3 (0.010)<br>IR-4 (0.019) & S-2 (0.038)<br>Red Sensitive Silver Iodobromide Emulsion (0.194 Ag), 4.1 mole % Iodide T-Grain (1.2 x 0.11 $\mu\text{m}$ )<br>Red Sensitive Silver Iodobromide Emulsion (0.236 Ag), 4.1 mole % Iodide T-Grain (0.91 x 0.11 $\mu\text{m}$ )<br>Gelatin (1.076)               |
| 11 Slow Cyan Layer:    | CC-1 (0.533) & S-2 (0.560)<br>IR-4 (0.026) & S-2 (0.052)<br>CM-1 (0.032)<br>B-1 (0.056) & S-3 (0.073)<br>Red Sensitive Silver Iodobromide Emulsion (0.463 Ag), 1.5 mole % Iodide T-Grain (0.54 x 0.06 $\mu\text{m}$ )<br>Red Sensitive Silver Iodobromide Emulsion (0.301 Ag) 4.1 mole % Iodide T-Grain (0.53 x 0.12 $\mu\text{m}$ )<br>Gelatin (1.679)               |
| 12 Antihalation Layer: | Gray Silver (0.135)<br>UV-1 (0.075), UV-2 (0.030), S-1 (0.042) S-4 (0.015)<br>YD-1 (0.034), MD-1 (0.018) & S-5 (0.018)<br>CD-1 (0.025) & S-2 (0.125)<br>R-1 (0.161), S-2 (0.261) & ST-2 (0.022)<br>Gelatin (2.04)                                                                                                                                                     |

Cellulose Triacetate Support



TABLE V-continued

## MULTILAYER FILM STRUCTURE

CC-1



CD-1



CM-1



IR-1



TABLE V-continued

## MULTILAYER FILM STRUCTURE

IR-2



IR-3



IR-4



TABLE V-continued

## MULTILAYER FILM STRUCTURE



TABLE V-continued

## MULTILAYER FILM STRUCTURE



TABLE V-continued

## MULTILAYER FILM STRUCTURE



The preceding examples are set forth to illustrate specific 30 embodiments of this invention and are not intended to limit the scope of the compositions, materials or methods of the invention. Additional embodiments and advantages within the scope of the claimed invention will be apparent to one skilled in the art.

The entire contents of the patents and other publications referred to in this specification are incorporated herein by reference.

What is claimed is:

1. A photographic element comprising a light-sensitive 40 silver halide emulsion layer having associated therewith a coupler based on a 1-aryl-3-arylpypyrazol-5-one or a 1-aryl-3-alkylpypyrazol-5-one ring and represented by formula I:

I 45



wherein:

X represents an aryl, alkyl, alkylamino, or arylamino group;

Y can be carbon or sulfur; m is 1 when Y is carbon and 60 2 when Y is sulfur;

R represents a halogen or an alkyl group; and o is 0 to 4, provided that two or more R substituents may join to form one or more additional rings;

Z is either (a) an aryl group represented as Ar<sup>3</sup>Q(n) where 65

Q represents n independently selected substituents bonded to the Ar<sup>3</sup> ring; and n is 0 to 5, provided that

two or more Q substituents may join to form one or more additional rings or (b) an alkyl group;

OAr<sup>4</sup> is an aryloxy group; and

P represents p independently selected substituents bonded to the OAr<sup>4</sup> aryloxy ring, provided that P may not be a nitro group ortho to the oxygen atom linking the aryloxy group to the 4-position of the pyrazolone ring; and p is 0 to 5, provided that two or more P substituents may join to form one or more additional rings;

provided that X and an R group may join to form an additional ring.

2. The element of claim 1 wherein Ar<sup>3</sup> is a phenyl group.

3. The element of claim 2 wherein Ar<sup>3</sup> is a p-chlorophenyl group.

4. The element of claim 2 wherein Ar<sup>3</sup> is a p-fluorophenyl group.

5. The element of claim 1 wherein OAr<sup>4</sup> is a phenoxy group.

6. The element of claim 5 wherein OAr<sup>4</sup> is a p-nitrophenoxy group.

7. The element of claim 5 wherein OAr<sup>4</sup> is a p-cyanophenoxy group.

8. The element of claim 1 wherein Y is carbon.

9. The element of claim 1 wherein Y is sulfur.

10. The element of claim 1 where X is 2,4-di(t-pentyl)phenoxymethyl group.

11. The element of claim 1 wherein X is 1-[2,4-di(t-pentyl)phenoxy]-1-propyl group.

12. The element of claim 1 wherein Z is a methyl group and OAr<sup>4</sup> is a p-nitrophenoxy group.

13. The element of claim 1 where Z is t-butyl group and OAr<sup>4</sup> is a p-nitrophenoxy group.

- 14. The element of claim 12 wherein Y is carbon.
- 15. The element of claim 13 wherein Y is carbon.
- 16. The element of claim 12 wherein Y is sulfur.
- 17. The element of claim 13 wherein Y is sulfur.
- 18. The element of claim 14 wherein X is 2,4-di(t-pentyl) 5 phenoxyethyl group.

- 19. The element of claim 15 wherein X is 1-(2,4-di(t-pentyl)phenoxy]-1-propyl group.
- 20. The element of claim 1 wherein P contains a photographically useful group (PUG).

\* \* \* \* \*